# EUROPEAN PATENT SPECIFICATION

(11) **EP 2 964 808 B1**
(45) Date of publication and mention of the grant of the patent: **01.05.2019**
(21) Application number: 13877283.5
(22) Date of filing: 30.12.2013
(51) Int. Cl.: C23C 4/06, C23C 4/18, C22C 21/00, C22C 1/04, C22C 1/10, B22F 9/08

(54) **THERMO-MECHANICAL FATIGUE RESISTANT ALUMINUM ABRADABLE COATING**
THERMOMECHANISCHE, ERMÜDUNGSBESTÄNDIGE UND ABREIBBARE ALUMINIUMBESCHICHTUNG
REVÊTEMENT ABRADABLE EN ALUMINIUM RÉSISTANT À LA FATIGUE THERMOMÉCANIQUE

(30) Priority: 06.03.2013 US 201361773344 P
(43) Date of publication of application: 13.01.2016
(73) Proprietor: United Technologies Corporation, Farmington, CT 06032 (US)
(72) Inventor: STROCK, Christopher W., Kennebunk, Maine 04043 (US)
(74) Representative: Dehns
(86) International application number: PCT/US2013/078183
(87) International publication number: WO 2014/137464

(56) References cited:
- EP-A1- 0 258 510
- EP-A2- 1 801 248
- WO-A2-2007/117279
- US-A- 4 836 982
- US-A- 5 434 210
- US-A1- 2004 057 832
- US-A1- 2007 141 369
- US-A1- 2009 297 720

## Description

### BACKGROUND

The present disclosure relates to a thermo-mechanical fatigue (TMF) resistant aluminum abradable coating which has particular utility as an outer air seal.

Compressor efficiency is related to blade tip clearance and outer air seal roughness. Coatings for the fan and the low pressure compressor are typically applied on titanium or iron based parts. The coefficient of thermal expansion (CTE) mismatch between the aluminum coating and the base metal (the titanium or iron) is almost a factor of two. This may lead to high compressive stresses in the coating during elevated temperature operation. With many thermal cycles from room temperature and back, the result is thermo-mechanical fatigue cracking and coating spallation.

Blades that mate with an aluminum seal may be titanium- or iron-based. During rub interaction, under certain conditions, metal is transferred to the blade tips. This may cause localized wear of the seal in what is known as record groove patterns. The result is increased average tip clearance and increased roughness in the air flow direction.

It is known in the art to form an aluminum based abradable coating made with hexagonal boron nitride. The problem with this type of coating however is that the hexagonal boron nitride is weak and does not bond well to the matrix.

EP 1 801 248 A discloses in an example a sealing composition made from a composite powder comprising 45 mass % boron nitride and 65 mass % of titanium diboride and having an average particle size of 15 - 30 µm. The powder is mixed with a fine powder of aluminum containing 12 mass % of silicon. An organic binder is mixed in with the metal and composite powder to form a slurry. The mixture is heated to about 150 °C and stir blended until the material is dried and an agglomerated powder is formed. The powder is then screened a size of 40 to 210 µm. The powder is sprayed with a plasma gun onto a substrate to a coating of 30 µm thickness.

It is desirable to control the coefficient of thermal expansion of the aluminum coating to be closer to the coefficient of thermal expansion of the base metal and thereby prevent thermo-mechanical fatigue related coating failure.

### SUMMARY

The invention is defined by an aluminum coating comprising an aluminum alloy matrix as claimed in claim 1, a process of applying the coating as claimed in claim 8, and a process of forming the aluminum alloy matrix as claimed in claim 12. Preferred embodiments are defined in dependent claims 2 to 7, and 9 to 11.

Other details of the thermo-mechanical fatigue resistant aluminum abradable coating are set forth in the following detailed description.

### DETAILED DESCRIPTION

As discussed above, there is disclosed an aluminum coating which has a coefficient of thermal expansion which more closely matches the coefficient of thermal expansion of the substrate to which the aluminum coating is applied.

The substrate to which the aluminum coating described herein may be applied may be formed from a titanium alloy or from an iron based alloy. For example, the substrate may be a fan casing or a casing for a compressor section of gas turbine engine.

The aluminum coating has an aluminum matrix formed from an aluminum alloy such as an aluminum-silicon alloy. The aluminum coating further includes fine particles in the range of 20 nm to 5 µm mean particle diameter of a low coefficient of thermal expansion (cte) material, which is defined as having a cte that is lower than that of the aluminum matrix, which are incorporated into the aluminum matrix. In a non-limiting embodiment, the fine particles may be in the range of from 20 nm to 2 µm in mean particle size. The inclusion of the fine particles of a low coefficient of thermal expansion material results in hardening, strengthening and coefficient of thermal expansion reduction. By controlling the amount of fine particles incorporated into the coating, one can control the coefficient of thermal expansion so as to reduce the coefficient of thermal expansion mismatch with the substrate to which the aluminum coating is applied. The amount of fine particles may also be controlled to provide other desirable coating properties.

The fine particles to be incorporated into the aluminum coating are boride particles. Only those particles which bond sufficiently well to the aluminum alloy matrix material and are capable of carrying a portion of the mechanical load and which act as a composite material are used in the aluminum coating described herein, such as aluminum boride particles and titanium boride particles.

Aluminum boride particles form high aspect ratio platelets when precipitated at a temperature of below about 650 degrees Centigrade. When aluminum boride particles are used, the technique used to manufacture the aluminum coatings must contain sufficient heating of the alloy constituents to fully dissolve any AlB₁₂ which tends to form at temperatures between 650 degrees Centigrade and 1550 degrees Centigrade depending on boron concentration. The formation of AlB₁₂ during cooling may be suppressed by quenching to below 650 degrees Centigrade. This can bed one by rapid cooling of the melt or passively as one of the characteristics of thermal spray coating in which molten particles are quench cooled upon impact with a surface. If desired, the thermal spray coating may be subsequently heat treated to a temperature of up to 650 degrees Centigrade. Aluminum boride is a desirable candidate due to its low cost, high thermal conductivity, low coefficient of thermal expansion, and good adhesion to the matrix. Aluminum boride at 20 vol% has been shown to increase the strength of aluminum by 80%.

Titanium boride is also a desirable candidate for the aluminum coating. When using titanium boride, the titanium boride particles may be incorporated into the aluminum matrix by precipitation from a quenched metastable solid solution. The titanium boride may have a ratio of titanium to boron which ranges from 1:1 to 1:4. It is also possible to include the titanium boride particles by mechanical alloying, agglomeration with the matrix alloy in a thermal spray feed stock powder, pressed and sintered.

The borides, such as titanium boride or aluminum boride, used as the fine particles may be present in a range of from 1.0 vol% to 33 vol%, balance aluminum matrix. In another non-limiting embodiment, the boride particles may be present in an amount from 10 to 25 vol%. In still another non-limiting embodiment, the boride particles may be present in an amount from 15 to 20 vol%.

The borides are dissolved in melt atomization to form a spray powder. Melt atomization of a boride containing aluminum alloy that quenches during atomization forms particles of a metastable solid solution. This allows deposition of solid or semi-solid particles and subsequent precipitation. The precipitation of undesirable phases may be suppressed as a result of rapid cooling rates. Alternatively, other powder manufacturing routes that result in powder with undesirable phases may be melted and solutionized during the spray coating operation. Either way, molten or softened particles may then be quench cooled during deposition. When an aluminum - titanium - boron alloy is used, titanium boride precipitates from a metastable quenched structure to form precipitates in the 20nm to 2.0 micron size range, depending on subsequent heat treat temperature. The heat treatment could be heating the aluminum coating at 625 to 650 degrees Centigrade for 2.0 hours.

The aluminum alloy matrix with fine particles is formed into a powder so that it can be applied on the substrate by a spray process such as thermal spraying. The fine particles may be included in the particles forming the aluminum alloy matrix material by agglomeration, alloying and precipitation, or ball milling and cold working. The amount of fine particles is a function of the desired coefficient of thermal expansion for the aluminum coating. Also, considerations of through thickness thermal gradient may be taken into account.

The aluminum coating is applied to the substrate by thermally spraying the matrix material with the incorporated fine particles. Hexagonal boron nitride as a pore making fugitive or soft filler material is added to the matrix material while it is being sprayed. The fugitive or soft filler material does not affect the coefficient of thermal expansion of the aluminum coating. To affect the coefficient of thermal expansion, the filler material would have to both bond with the aluminum matrix and have sufficient elastic modulus to at least partially elastically constrain the aluminum matrix. The elastic modulus of the filler material may be higher than that of aluminum. Fugitives and fillers like hexagonal boron nitride, polyester, and Lucite ® are candidates for affecting the abradability of the aluminum coating and may be used to offset the strengthening of the matrix material by the fine particles. The coating is made from an aluminum alloy containing 70.4 wt% aluminum, 13.8 wt% titanium, 9.6 wt% silicon, and 6.2 wt% boron and hexagonal boron nitride to produce a coating of 40 volume % aluminum alloy, 50 volume % hBN and 10% porosity. The titanium boride particles may be precipitated from a quenched metal alloy with heat treatment at 625 to 650 degrees Centigrade for 2.0 hours.

While the aluminum coating particles are sprayed onto the substrate, the sprayed particles may be quenced by conduction of heat to the coating and substrate cooling the particles. After quenching, the substrate with the sprayed particles may be subjected to a heat treatment in the range of from 625 to 650 degrees Centigrade for 2.0 hours.

The benefits of the abradable coating described herein include reduced coefficient of thermal expansion and thermo-mechanical fatigue. This results in a more stable part shape with temperature change and improved coating durability. The filler material also helps to reduce metal transfer to blades during low interaction rate sliding contact wear and result in tighter tip clearance and a smoother coating. As compared to choosing a conventional alloy that has a lower coefficient of thermal expansion, the technique described herein does not increase the incipient melting point of the coating. With regard to the alloy mentioned above, this is because the titanium and boride constituents fully precipitate as a high melting point phase. As a result, the blade tip temperature, particularly of a titanium blade tip, during rub is still limited to the melting point of aluminum. This helps reduce the risk of a titanium fire.

The coatings described herein have good adhesion between the fine particles and the matrix.

There has been described herein a thermo-mechanical fatigue resistant aluminum abradable coating. While the coating has been described in the context of specific embodiments thereof, other unforeseeable alternatives, modifications, and variations may become apparent to those skilled in the art having read the foregoing description. Accordingly, it is intended to embrace those alternatives, modifications, and variations as fall within the broad scope of the appended claims.

## Claims

1. An aluminum coating to be deposited on a substrate having a first coefficient of thermal expansion, said aluminum coating comprising an aluminum alloy matrix and boride particles having a low coefficient of thermal expansion incorporated into said matrix; **characterized in that** said coating is made of an aluminum alloy containing 70.4 wt.% aluminum, 13.8 wt.% titanium, 9.6 wt.% silicon, and 6.2 wt.% boron and hexagonal boron nitride (hBN) to produce a coating of
(i) 40 volume % of aluminum alloy;
ii) 50 % vol. hexagon boron nitride (hBN); and
iii) 10 % vol. porosity.

2. The aluminum coating of claim 1, wherein said particles are aluminum boride particles.

3. The aluminum coating of claim 1, wherein said particles are titanium boride particles.

4. The aluminum coating of claim 3, wherein said titanium boride particles have a ratio of titanium to boron in the range of 1:1 to 1:4.

5. The aluminum coating of any preceding claim, wherein said particles are present in an amount from 1.0 to 33 vol%.

6. The aluminum coating of any of claims 1 to 4, wherein said particles are present in an amount of from 10 to 25 vol%.

7. The aluminum coating of any of claims 1 to 4, wherein said particles are present in an amount of 15 to 20 vol%.

8. A process for applying an aluminum coating of any preceding claim to a part comprising the steps of:
providing a part;
forming a powder containing said aluminum alloy matrix and boride particles having a low coefficient of thermal expansion bonded to said aluminum matrix; and
thermally spraying said powder onto said part.

9. The process of claim 8, wherein said part providing step comprises providing a part formed from a titanium based alloy or an iron based alloy.

10. The process of claim 8 or 9, wherein said powder forming step comprises melt atomization of a boride containing aluminum alloy and quenching the boride containing aluminum alloy during atomization to form particles of a metastable solid solution.

11. The process of claim 8, 9 or 10, further comprising subjecting said aluminum coating to a heat treatment in the range of from 625 to 650 degrees Centigrade for 2.0 hours.

12. A process for forming an aluminum alloy matrix containing fine boride particles comprising the steps of:
melt atomizing a boride containing aluminum alloy containing 70.4 wt.% aluminum, 13.8 wt.% titanium, 9.6 wt.% silicon, and 6.2 wt.% boron; and
quenching the boride containing aluminum alloy during atomization to form particles of a metastable solid solution.

## Patentansprüche

1. Aluminiumbeschichtung, die auf einem Substrat abgeschieden werden soll, das einen ersten Wärmeausdehnungskoeffizienten aufweist, wobei die Aluminiumbeschichtung eine Aluminiumlegierungsmatrix und Boridpartikel aufweist, die einen niedrigen Wärmeausdehnungskoeffizienten aufweisen, der in die Matrix eingebunden ist;
**dadurch gekennzeichnet, dass** die Beschichtung aus einer Aluminiumlegierung hergestellt ist, die 70,4 Gew.-% Aluminium, 13,8 Gew.-% Titan, 9,6 Gew.-% Silicium und 6,2 Gew.-% Bor und hexagonales Bornitrid (hBN) enthält, um eine Beschichtung zu produzieren, die Folgendes enthält:
(i) 40 Vol.-% Aluminiumlegierung;
(ii) 50 Vol.-% hexagonales Bornitrid (hBN); und
(iii) 10 Vol.-% Porosität.

2. Aluminiumbeschichtung nach Anspruch 1, wobei die Partikel Aluminiumboridpartikel sind.

3. Aluminiumbeschichtung nach Anspruch 1, wobei die Partikel Titanboridpartikel sind.

4. Aluminiumbeschichtung nach Anspruch 3, wobei die Titanboridpartikel ein Verhältnis von Titan zu Bor in dem Bereich von 1:1 bis 1:4 aufweisen.

5. Aluminiumbeschichtung nach einem der vorhergehenden Ansprüche, wobei die Partikel in einer Menge ab 1,0 bis 33 Vol.-% vorhanden sind.

6. Aluminiumbeschichtung nach einem der Ansprüche 1 bis 4, wobei die Partikel in einer Menge von ab 10 bis 25 Vol.-% vorhanden sind.

7. Aluminiumbeschichtung nach einem der Ansprüche 1 bis 4, wobei die Partikel in einer Menge von 15 bis 20 Vol.-% vorhanden sind.

8. Verfahren zum Aufbringen einer Aluminiumbeschichtung nach einem der vorhergehenden Ansprüche auf ein Teil, das die folgenden Schritte umfasst:
Bereitstellen eines Teils;
Bilden eines Pulvers, das die Aluminiumlegierungsmatrix und Boridpartikel, die einen niedrigen Wärmeaufdehnungskoeffizienten aufweisen und die an die Aluminiummatrix gebunden sind, enthält, und
thermisches Aufspritzen des Pulvers auf das Teil.

9. Verfahren nach Anspruch 8, wobei der Schritt des Bereitstellens des Teils das Bereitstellen eines Teils umfasst, das aus einer auf Titan basierenden Legierung oder aus einer auf Eisen basierenden Legierung gebildet ist.

10. Verfahren nach Anspruch 8 oder 9, wobei der Schritt des Bildens des Pulvers Schmelz-Zerstäubung eines Borids, das eine Aluminiumlegierung enthält, und Quenchen des die Aluminiumlegierung enthaltenden Borids während der Zerstäubung umfasst, um Partikel einer metastabilen Feststofflösung zu bilden.

11. Verfahren nach Anspruch 8, 9 oder 10, das ferner Aussetzen der Aluminiumbeschichtung gegenüber einer Hitzebehandlung in dem Bereich von 625 bis 650 Grad Celsius für 2,0 Stunden umfasst.

12. Verfahren zum Bilden einer Aluminiumlegierungsmatrix, die feine Boridpartikel enthält, das die folgenden Schritte umfasst:
Schmelz-Zerstäuben einer Borid enthaltenden Aluminiumlegierung, die 70,4 Gew.-% Aluminium, 13,8 Gew.-% Titan, 9,6 Gew.-% Silicium und 6,2 Gew.-% Bor umfasst; und
Quenchen der Borid enthaltenden Aluminiumlegierung während der Zerstäubung, um Partikel einer metastabilen Feststofflösung zu bilden.

## Revendications

1. Revêtement en aluminium qui doit être déposé sur un substrat ayant un premier coefficient de dilatation thermique, ledit revêtement en aluminium comprenant une matrice en alliage d'aluminium et des particules de borure ayant un faible coefficient de dilatation thermique incorporées dans ladite matrice ;
**caractérisé en ce que** ledit revêtement est composé d'un alliage d'aluminium contenant 70,4 % en poids d'aluminium, 13,8 % en poids de titane, 9,6 % en poids de silicium et 6,2 % en poids de bore et de nitrure de bore hexagonal (hBN) pour produire un revêtement de
(i) 40 % en volume d'alliage d'aluminium ;
(ii) 50 % en volume de nitrure de bore hexagonal (hBN) ; et
(iii) 10 % en volume de porosité.

2. Revêtement en aluminium selon la revendication 1, dans lequel lesdites particules sont des particules de borure d'aluminium.

3. Revêtement en aluminium selon la revendication 1, dans lequel lesdites particules sont des particules de borure de titane.

4. Revêtement en aluminium selon la revendication 3, dans lequel lesdites particules de borure de titane ont un rapport de titane sur bore dans la plage de 1:1 à 1:4.

5. Revêtement en aluminium selon une quelconque revendication précédente, dans lequel lesdites particules sont présentes dans une quantité de 1,0 à 33 % en volume.

6. Revêtement en aluminium selon l'une quelconque des revendications 1 à 4, dans lequel lesdites particules sont présentes dans une quantité de 10 à 25 % en volume.

7. Revêtement en aluminium selon l'une quelconque des revendications 1 à 4, dans lequel lesdites particules sont présentes dans une quantité de 15 à 20 % en volume.

8. Procédé pour appliquer un revêtement en aluminium selon une quelconque revendication précédente à une pièce comprenant les étapes suivantes :
la fourniture d'une pièce ;
la formation d'une poudre contenant ladite matrice en alliage d'aluminium et des particules de borure ayant un faible coefficient de dilatation thermique liées à ladite matrice en aluminium ; et
la pulvérisation thermique de ladite poudre sur ladite pièce.

9. Procédé selon la revendication 8, dans lequel ladite étape de fourniture de pièce comprend la fourniture d'une pièce formée à partir d'un alliage à base de titane ou d'un alliage à base de fer.

10. Procédé selon la revendication 8 ou 9, dans lequel ladite étape de formation de poudre comprend l'atomisation à chaud d'un alliage d'aluminium contenant du borure et le refroidissement de l'alliage d'aluminium contenant du borure au cours de l'atomisation pour former les particules d'une solution solide métastable.

11. Procédé selon la revendication 8, 9 ou 10, comprenant en outre le fait de soumettre ledit revêtement en aluminium à un traitement thermique dans la plage de 625 à 650 degrés centigrades pendant 2,0 heures.

12. Procédé pour former une matrice en alliage d'aluminium contenant de fines particules de borure comprenant les étapes suivantes :
atomisation à chaud d'un alliage d'aluminium contenant du borure, contenant 70,4 % en poids d'aluminium, 13,8 % en poids de titane, 9,6 % en poids de silicium et 6,2 % en poids de bore; et
refroidissement de l'alliage d'aluminium contenant du borure au cours de l'atomisation pour former des particules d'une solution solide métastable.
